

# UNITED STATES PATENT OFFICE.

ROYALL OSCAR EUGENE DAVIS, OF CHAPEL HILL, NORTH CAROLINA, ASSIGNOR OF ONE-  
THIRD TO RISDEN T. ALLEN, OF CHAPEL HILL, NORTH CAROLINA.

## COMPOSITION FOR COPYING-PADS.

No. 908,967.

Specification of Letters Patent.

Patented Jan. 5, 1909.

Application filed March 12, 1908. Serial No. 420,739.

*To all whom it may concern:*

Be it known that I, ROYALL OSCAR EUGENE DAVIS, a citizen of the United States, and a resident of Chapel Hill, in the county 5 of Orange and State of North Carolina, have invented a new and Improved Composition for Copying-Pads, of which the following is a full, clear, and exact description.

My invention relates to compositions for 10 copying pads, my more particular purpose being to produce a composition tablet having certain desirable properties hereinafter described, and used for the purpose of making repeated copies of characters made by ink 15 upon paper. As is well understood in this art, it is a common practice to prepare a pad of material more or less absorbent, the pad having the form of a smooth tablet, capable of transferring copying ink to a large number 20 of successive sheets of paper so as to reproduce a number of fac-similes of the original paper to be copied. In preparing such tablets, it is desirable that the material used shall not be too hard, on the one hand, or so 25 soft as to crumble or become distorted, on the other hand. It is also desirable that the material when made into tablet form, shall be capable of absorbing the copying ink, and yet incapable of absorbing it to such an extent 30 that it becomes lost in the composition.

I find it very desirable in making and using tablets for the purpose above indicated, to render the tablet capable of conforming to various conditions due to changes in the atmosphere, and particularly to the amount of moisture present. I accordingly make my tablet of such composition that, in case the atmosphere happens to be excessively dry or excessively damp, the tablet, because of its 35 composition, undergoes slight changes in condition, so that the amount of moisture present in the atmosphere is not allowed to interfere with the proper operation of the tablet or of the materials of which it is composed. I take a metal-lined wooden tray and fill my preparation into it so as to bring the surface of the composition flush with the upper level of the tray, and allow the material 40 to remain in the tray thereafter. The composition is made of the following materials in the proportions by weight as stated: aluminum oxid, 78 parts, silica (in the form of sand), 92 parts, potassium carbonate, 1 part, calcium sulfate, 10 parts, and glycerin, 64

parts. These ingredients are thoroughly 55 mixed together, a little water is poured in with them, and the whole kneaded like dough and placed in the metal-lined wooden tray so as to fill it completely as above described, the upper level of the composition being smoothed 60 off for use as a copying surface. In order to use the tablet thus made, I place upon it, face downwardly, a sheet of paper from which the written words or other intelligible characters are to be copied. Pressure is applied in the usual manner so that the ink from the paper is absorbed slightly by the upper surface of the tablet. The pressure is continued for about a minute; the paper is then removed and replaced by a blank sheet 70 of paper, to which pressure is applied as before. The sheet last mentioned, being removed, will show on its under face a fac-simile of the characters appearing upon the original sheet. A considerable number of copies 75 can thus be made, the general action of the tablet after its formation, being substantially similar to that of other tablets heretofore used.

As is well known potassium carbonate 80 varies in composition with regard to the water content, but the amount of water it can attract and hold varies with the changes 85 in the atmosphere. This is true because the vapor pressure of potassium carbonate varies with the temperature. Ordinarily it contains 3 molecules of water at a temperature of 32° with the power of attracting more water from the atmosphere until it forms a solution, but at 100° it is capable of holding only one molecule of water, and at a somewhat higher temperature its vapor pressure is so great that it can hold no water. Hence the composition of the water content 90 will vary materially for a small range of temperature. For this reason when the temperature rises and the composition tends to soften due to the greater fluidity of glycerin at the higher temperature, such tendency is overcome by the potassium carbonate giving 95 up some of the water attracted at a lower temperature.

Having thus described my invention, I claim as new and desire to secure by Letters Patent:

1. A composition for copying tablets containing by weight, the following ingredients; aluminum oxid, 78 parts, silica 92 parts,

potassium carbonate 1 part, calcium sulfate 10 parts, and glycerin 64 parts.

2. A composition for copying tablets consisting of aluminum oxid, silica, potassium carbonate, calcium sulfate, and glycerin in substantially the proportions set forth.

3. A composition for copying tablets composed of substances capable of absorbing and transmitting ink combined with potassium

carbonate in substantially the proportions set forth.

In testimony whereof I have signed my name to this specification in the presence of two subscribing witnesses.

ROYALL OSCAR EUGENE DAVIS.

Witnesses:

CLYDE EUBANKS,

RISDEN T. ALLEN.